

Oct. 10, 1939.

F. M. CLARK

2,175,877

LIQUID COMPOSITION

Filed Sept. 30, 1936

Fig. 1.



Fig. 2.



Inventor:  
Frank M. Clark,  
by Harry E. Dunham  
His Attorney.

## UNITED STATES PATENT OFFICE

2,175,877

## LIQUID COMPOSITION

Frank M. Clark, Pittsfield, Mass., assignor to  
 General Electric Company, a corporation of  
 New York

Application September 30, 1936, Serial No. 103,313

7 Claims. (Cl. 87—9)

The present application comprises liquid compositions of neutral oily consistency characterized by low viscosity at low temperature and more uniform viscosity-temperature relation than is normally associated with ordinary mineral oil or vegetable oil compositions, such as are used for lubricating, electrical insulating and other industrial purposes.

It is one of the objects of my invention to provide oily liquids suitable for cooling and dielectric purposes in electric devices, such as transformers.

Another object of my invention is to provide low viscosity liquids of superior characteristics for use in electric cables of the liquid-filled type,

It is a further object of my invention to provide an improved liquid dielectric impregnant for capacitors whereby the electric capacity is materially increased and the electrical operation at low temperature improved.

Still another object is to provide an improved liquid dielectric for arc interrupting devices. Many arc interruption devices operate efficiently only when they are provided with liquids of low viscosity. This is especially true for those arc interrupting devices which are constructed to open an electric circuit within a definite number of alternations of voltage on alternating current circuits. Even the lowest viscosity mineral oil having a required resistance to ignition within a prescribed limit of temperature has such increased viscosity at temperatures below room temperature, especially at temperatures as low as —30° C. and lower, that it constitutes a serious obstacle in the operation of such devices.

It is also an object of my invention to provide compositions of superior lubrication characteristics. My improved liquid compositions not only have minimum viscosity change with temperature but also have as well superior extreme pressure lubrication characteristics as will hereinafter be shown. As a consequence of my invention I have provided lubricant and dielectric compositions of low pour point.

Other and important objects and applications of my invention will appear hereinafter.

The essential ingredients of my novel compositions are oily liquid materials of mineral or vegetable or synthetic origin in combination with one or more alkyl phosphates, this term being used to designate such phosphates in their ordinary, unsubstituted form. Such compositions normally should contain by weight about 5 to 25 per cent of the alkyl phosphate, but such ingredient is not necessarily restricted to such limits.

Examples of oily materials constituting an essential ingredient of the compositions of this invention are mineral oils of the type in general use in electric transformers, cables, capacitors, arc interrupting devices and the like; mineral oils in general lubrication use for automotive and other mechanical devices; vegetable oils such as castor and linseed oils, synthetic oily liquids of the ester type (for example, butyl stearate, or tartrate or phthalate), or other oily ester derivatives of the alkyl or phenyl hydrocarbon nucleii, or chlorinated oil liquids such as the chlorodiphenyl, chlorodiphenyl oxides and others hereinafter designated.

As illustrative of the second ingredient used in combination with the foregoing materials, are alkyl phosphate esters, such as the ethyl, propyl or butyl esters, or combinations thereof. Such esters may be designated, generally, by the empirical formula  $RPO_4$ , wherein R comprises an alkyl radical containing not exceeding four (4) carbon atoms. For some purposes tributyl phosphate is preferred.

In the accompanying drawing Fig. 1 is a graph showing the viscosity characteristics of mineral oil compositions embodying my invention over a range of temperatures; and Fig. 2 is a graph showing the viscosity variation of a composition embodying my invention with changes of proportion of the ingredients.

In the graph of Fig. 1 temperature values are plotted as abscissae over a range from about 50° C. down to the lowest temperatures encountered climatically. The curve A shows the viscosities over a range of about 100° of a mixture by weight of 25 per cent of tributyl phosphate and 75 per cent of a mineral oil. The data given for a composition containing a light mineral oil such as commercially designated as "10-C Oil". The viscosity of the mixture changes but little as the temperature falls from 50° C. to about 20° C. and then as the temperature continues to fall to about —40° C. the viscosity rises only to 600 seconds Saybolt. The mineral oil unassociated with modifying ingredients on the other hand begins to rapidly increase in viscosity at about 0° C. Its viscosity-temperature characteristic is shown by curve B as rising to about 10,000 seconds Saybolt at —40° C.

As shown by curve C a mixture of equal parts by weight of tributyl phosphate and mineral oil has an even lower viscosity at very low temperatures. At —45° C. the viscosity of this mixture is still below 400 seconds Saybolt.

A particular composition adapted for use in

transformers, electric cables and arc interrupting devices consists of 75 per cent mineral oil of the type normally used in electric transformers and 25 per cent by weight of the tributyl phosphate. Such a composition has the following properties:

|    |                          |                    |           |         |
|----|--------------------------|--------------------|-----------|---------|
|    | Viscosity at -40° C.     | 590                | seconds   | Saybolt |
|    |                          |                    | Universal |         |
|    | Viscosity at +37.8° C.   | 46                 | seconds   | Saybolt |
|    |                          |                    | Universal |         |
| 10 | Viscosity at 100° C.     | 35                 | seconds   | Saybolt |
|    |                          |                    | Universal |         |
|    | Gravity at 15.5/15.5° C. | .905               |           |         |
|    | Condition                | Clear              |           |         |
| 15 | Flash point              | 136° C.            |           |         |
|    | Burn point               | 168° C.            |           |         |
|    | Pour point               | Lower than -50° C. |           |         |
|    | Dielectric strength      | 33 kv.             |           |         |

- 20 Because of its improved viscosity-temperature characteristics coupled with the higher burn point than that normally associated with the usual transformer oil, such a composition has been found particularly well adapted for electrical 25 insulating use in electric devices. One of my improved compositions when used in an arc interrupting device in which speed of circuit interruption is of major importance resulted in a speed of operation at temperatures in the range 30 of about -40 to -50° C., approximately 66 per cent over the normal speed obtained with the low viscosity mineral oil which had been used.

Compositions comprising mixtures of castor oil and tributyl phosphate further illustrate the present improvement. The relatively high pour point of castor oil (about -10° C.) limits its use as a lubricant and as a liquid dielectric material in electrical devices. By the addition of tributyl phosphate, or equivalent ester phosphate, to castor oil the viscosity at low temperatures is materially decreased. In the following table are compared viscosities at various temperatures and also pour point of two such mixtures with castor oil such as ordinarily obtained, that is, unmixed with any modifier (designated as product 3):

| Product | Castor oil | Tributyl phosphate | Pour point | Viscosity |       |     |        |        |
|---------|------------|--------------------|------------|-----------|-------|-----|--------|--------|
|         |            |                    |            | 100°      | 37.8° | 25° | -17°   | -25°   |
| 50      | Percent    | Percent            |            | °C.       | °C.   | °C. | °C.    | °C.    |
| 1       | 75         | 25                 | -35        | 64        | 378   | 660 | 52,000 | (1)    |
| 2       | 50         | 50                 | -50        | 47        | 128   | 196 | (1)    | 36,000 |
| 3       | 100        | 0                  | -10        | 120       | 1,350 | (1) | (1)    | (1)    |

1 Viscous. 2 Not measured. 3 Semisolid.

In place of a mineral or vegetable oil other liquid oily materials having a viscosity characteristic suitable for use for lubricating or dielectric purposes may be used in compositions embodying my invention. For example, I may employ as the oily constituent or base liquid chlorinated diphenyl, or liquid chlorinated diphenyl oxide, either with or without mineral oil. In my prior 60 Patent 2,037,686 patented April 14, 1936, I have described compositions of mineral oil and chlorinated diphenyl. I prefer to employ liquid chlorinated diphenyl compound containing about 54 per cent chlorine (corresponding substantially 65 to composition to pentachlor diphenyl), although some chlorinated compounds of lower and higher chlorine content may be present. As described in my prior Patent 2,041,594, patented May 19, 1936, compositions such as are ordinarily obtainable on the market consist of a mixture of

various isomers of pentachlor diphenyl. Such mixtures remain liquid at a lower temperature than a composition consisting of but a single isomer. Pentachlor diphenyl as ordinarily prepared, is a viscous liquid having a viscosity of about 48 to 50 seconds Saybolt at 100° C. and about 11,000 seconds Saybolt at 25° C. The pour point of this product is approximately 10° C.

When this material is compounded with even as little as 5 to 10 per cent by weight of tributyl phosphate, then the low temperature characteristics are remarkably changed. The viscosity is lowered materially by the presence of even a few per cent of alkyl phosphate, as shown in Fig. 2, which shows a graph D of the relation of viscosity at 25° C. of pentachlor diphenyl containing various proportions of tributyl phosphate.

Decreased viscosity of these compositions is accompanied by lowered pour points as shown in the following tabulation showing the pour points of three mixed products compared with chlorinated diphenyl (product 4) unassociated with phosphate ester:

| Product | Chlor diphenyl | Tributyl phosphate | Pour point |
|---------|----------------|--------------------|------------|
|         | Percent        | Percent            | °C.        |
| 4       | 100            | 0                  | +10        |
| 5       | 85             | 15                 | -10        |
| 6       | 75             | 25                 | -22        |
| 7       | 50             | 50                 | -50        |

Such mixtures are of particular utility as impregnants in capacitors. A given capacitor containing kraft paper when impregnated with pentachlor diphenyl as described in my prior Patent 2,041,594 (product 4) has a capacity of 5 microfarads. When product 6 (25 per cent of tributyl phosphate) is introduced in its place in such capacitor, the capacity is found to be 8 microfarads. When product 7 is employed the capacity is still further increased to approximately 11 microfarads. At temperatures below about 0° C. the capacity of capacitors impregnated with chlorinated diphenyl falls, due to solidification, to about 75 per cent of their original values. The drop in capacity of capacitors impregnated with mixtures containing tributyl phosphate is eliminated down to temperatures as low as the pour point of the mixtures.

In place of chlorinated diphenyl other similar compounds may be used as the oily base. For example, I may use chlorinated diphenyl ketone (described in U. S. Patent 2,012,301 of August 27, 1935) or chlorinated polyphenyl methane (described in U. S. Patent 2,012,302) or chlorinated dibenzyl (described in U. S. Patent 2,033,612, patented March 10, 1936) or chlorinated diphenyl oxide (described in my pending application Serial No. 73,595 filed April 9, 1936). All of these chlorinated compounds may be considered for the purpose of this invention as being chlorinated derivatives of diphenyl.

Illustrative of the lubricant use of my improved compositions are mixtures made up in part of a lubricant mineral oil having a viscosity of 100 seconds Saybolt Universal at 100° C. and of approximately 1200 to 1400 seconds at 37.8° C. Such a composition when including 25 per cent tributyl phosphate by weight has a viscosity of 261 seconds at 37.8° C., a reduction of about 82 percent. When containing 50 per cent tributyl phosphate, the viscosity is reduced at 37.8° C. to less than 6 per cent of the normal oil viscosity. Such admixtures containing tributyl

phosphate exhibit improved extreme pressure lubrication. With the selected lubricant oil the maximum load-carrying capacity was determined as 325 pounds for given conditions in a 5 Timken lubricant tester. With only 5 per cent by weight tributyl phosphate present the load-carrying capacity was increased to greater than 1,000 pounds. Similar increased load-carrying capacity was observed for mixtures containing 10 triethyl phosphate.

As a further illustration of the increase in the lubrication characteristics produced by compositions embodying my invention, the coefficient of friction and unit pressure values obtained at the 15 time of seizure of such compositions tested in the Timken tester are given in the following table from which the improved characteristics of my new compositions are evident:

| 20                                                  | Product         | Coefficient of friction | Unit pressure at seizure |
|-----------------------------------------------------|-----------------|-------------------------|--------------------------|
| Lubricant oil                                       | 0.102           | 2,355 lbs./sq. in.      |                          |
| Lubricant oil plus 5 percent tributyl phosphate.    | Less than .076* | Greater than 19,000.*   |                          |
| 25 Lubricant oil plus 5 percent triethyl phosphate. | Less than .051* | Greater than 20,000.*   |                          |

\*Limit of test machine. Actual lubricant breakdown and seizure of rubbing surfaces did not occur.

What I claim as new and desire to secure by 30 Letters Patent of the United States is:

1. A composition of matter consisting of vegetable oil and from 25 to 50 per cent by weight of the whole of an alkyl phosphate ester having the empirical formula  $RPO_4$ , where R comprises an 35 alkyl radical containing not exceeding four carbon atoms.

2. A composition of matter consisting of mineral oil and from 25 to 50 per cent by weight of the whole of an alkyl phosphate ester having the 40 empirical formula  $RPO_4$ , where R comprises an

alkyl radical containing not exceeding four carbon atoms.

3. A composition of matter consisting of an oily chlorinated aryl compound selected from the group consisting of chlorinated diphenyl derivatives and from 25 to 50 per cent by weight of the whole of an alkyl phosphate ester having the empirical formula  $RPO_4$ , where R comprises an alkyl radical containing not exceeding four carbon atoms. 5

4. A composition of matter consisting of pentachlor diphenyl and from 25 to 50 per cent by weight of the whole of an alkyl phosphate ester having the empirical formula  $RPO_4$ , where R comprises an alkyl radical containing not exceeding four carbon atoms. 10

5. A composition of matter consisting of castor oil and from 25 to 50 per cent by weight of the whole of an alkyl phosphate ester having the empirical formula  $RPO_4$ , where R comprises an alkyl radical containing not exceeding four carbon atoms. 20

6. A composition of matter consisting of mineral oil and from 25 to 50 per cent by weight of the whole of tributyl phosphate. 25

7. A liquid composition having a low and substantially uniform viscosity over a range of temperatures below  $0^\circ C.$ , said composition consisting by weight of a liquid, oily organic lubricant or dielectric compound of lubricating oil range 30 of viscosity, said base normally tending to become highly viscous at temperatures below  $0^\circ C.$ , and about 25 to 50 percent of an alkyl phosphate ester having the empirical formula  $RPO_4$ , where R comprises an alkyl radical containing not exceeding four carbon atoms, said phosphate ester being incorporated with the said oily base for the purpose of decreasing the viscosity of the latter at temperatures below  $0^\circ C.$  35

FRANK M. CLARK. 40